

April 27, 1943.

H. E. WALTER

2,317,504

ARTIFICIAL FIBER BOARD

Filed Feb. 3, 1940

2 Sheets-Sheet 1

*Fig. 1*



Inventor  
Henry E. Walter  
by W. Barrett Jones  
Attorney.

April 27, 1943.

H. E. WALTER

2,317,504

ARTIFICIAL FIBER BOARD

Filed Feb. 3, 1940

2 Sheets-Sheet 2



Fig. 1

Fig. 3



Fig. 2



Inventor  
Henry E. Walter  
by W. Barrett Jones,  
Attorney

## UNITED STATES PATENT OFFICE

2,317,504

## ARTIFICIAL FIBER BOARD

Henry E. Walter, Cloquet, Minn., assignor to  
 Wood Conversion Company, Cloquet, Minn., a  
 corporation of Delaware

Application February 3, 1940, Serial No. 317,063

5 Claims. (Cl. 41—24)

The present invention relates generally to marking temporarily plastic material in the process of manufacture to produce permanent markings. It has particular reference to the manufacture of fibrous felts, such as thick paper or artificial board to give decorative surfaces.

The use of artificial board for walls in certain places is limited by the fact that the common boards giving a desirable fibrous texture are too soft at the surface to resist scarring and scuffing, and are not sufficiently resistant to water to avoid spotting and to permit washing. Thus, for example, in the position of wainscot, boards of desirable decorative appearance lack qualities for such usage. The present invention aims also to produce wall boards which are suitable for use as decorative wainscot.

One object of the present invention is to produce intaglio impressions not of a definite pattern, but of a characteristic appearance in non-repetitive form; and to provide a means for that end.

Another object of the invention is to produce such boards with a hard surface which is resistant to spotting with water, to marring and scuffing, and which may be washed.

A particular object is to produce a decorative wainscot panel of the fibrous wallboard type.

The invention will be described with particular reference to artificial board made from an aqueous slurry of fibers, but it is to be understood, and it will be pointed out, that it has other applications; and that the device of the invention, and the manner of using it may vary considerably. Having reference to the accompany drawings, the invention will be illustrated and explained as it is applied in marking artificial board.

In the drawings:

Fig. 1 is a reproduction of a photographed picture of the surface of a wallboard panel made by the present invention.

Fig. 2 is a diagrammatic representation of the marking means.

Fig. 3 is an edge view more or less diagrammatic, of the means of Fig. 2.

Fig. 4 is a longitudinal vertical section of a machine for continuously marking a continuously formed web of wallboard.

In order to attain a non-repetitive pattern the impression means is multiple and each element is in part mobile and free to assume different positions. Each element is also in part constrained and fixed in part with respect to a carrier of the multiple elements, so that there is produced by the constraint, a general identity, or in-

dividual character in the design, and a pleasing non-repetitive variation in the design produced by the mobile parts.

This is readily accomplished where a design of lines is desired, by having one or more carrier elements to which a multiplicity of strands or cords is attached at points spaced along the strands or cords, each strand or cord being loose relative to the carrier between each two adjacent spaced points of attachment to the carrier, the looseness being due both to non-attachment to the carrier and to the cord or strand having a length greater than the distance measured in the carrier between adjacent points of attachment. Therefore, when the carrier is taut, the strands are not taut, and they may assume any free position between the points of attachment.

The carrier is one or more elements adapted to be pulled taut in one direction. The carrier is preferably a sheet backing. It may be a felt, or canvas, or rigid or flexible net, or merely be a plurality of parallel cords without lateral connections between them in the area used for impressions. The latter arrangement, and a coarse netting, can therefore be used in a taut position with varying widths coverable by the same backing, giving a finer or coarser pattern in the lateral direction.

The strands or cords may be of fiber, such as rope, yarn or cord, or flexible wire or even rubber, and the latter may be smooth or marked, as desired. One strand, for example, may be attached to the backing at evenly spaced intervals in a straight line, running generally in the direction of the taut backing, or definitely angular to it, or in some irregular line. Other cords may have an exactly similar attachment, and all points of attachment be arranged in parallel lines across the taut length. Some may be staggered with respect to others. There may be strands across the taut length. These may be attached to the backing, or even be a part of the backing, as where a coarse net is used, and not stretched laterally when it is pulled taut lengthwise.

In other words, the character of the backing, or the manner in which it is applied as a carrier, coupled with the pattern of the fixed points of attachment, is the means to provide the desired character or general identity to a design. The manner in which the cords or strands are free to assume different positions, is the cause of variation in the pattern, and the particular cause of a non-repetitive pattern.

In order to avoid showing the many possible variations of the pattern, one illustrative form

is selected, which gives a pleasing effect. In Fig. 2 there is shown a carrier which is a coarse net having a warp of heavy cords 10 adapted to be pulled taut to apply the carrier. Lighter weight transverse cords 11 are shown and at the intersections, any type of connection may be applied. When the net is expanded laterally to the full permissible width the transverse cords 11 will be taut, but for the purpose of illustration the net is shown slightly contracted laterally with a taut warp, whereby the transverse cords between the warp cords are irregularly arranged, and will make a variable design where they may penetrate the plastic material.

In Fig. 3 the diagrammatic block 12 indicates the edge of a carrier, and the single cord 13 thereon is representative of the strands which make the design. Cord 13 is shown with three spaced attachments 14, 15 and 16, of which 15 and 16 are points, while 14 is a length of cord 13 secured to carrier 12. On any carrier, the places of attachment, like 14 and 15, may be repetitive or non-repetitive in design. The repetitive design for attachment may be such as to give always an individual characteristic to the resulting effect, with uncontrollable variations from the loose parts. In Fig. 2, the strands or cords are designated 17, and the places of attachment are points 18, in a row across or otherwise disposed on the backing. Each strand 17 is shown with its series of spaced attachments aligned, not in a straight line, but in staggered relation, with looseness of strand between adjacent points in the taut carrier. Thus the strands may fall into wavy lines generally, but not mathematically or regularly, or repeatedly. From the foregoing it is obvious how the arrangement may be varied.

Where the carrier or backing is a flexible sheet relatively closed, like canvas, the strands are located on the impressing surface thereof. But where the carrier is more open, like a net, the strands may be on either side thereof, or both sides. Where the strands cross the net on the non-impressing side, the cords of the net may be utilized as part of the impression means. Likewise, the cords of the net may function where they are exposed on the impression side, between strands 17.

Fig. 4 represents one way in which such an impression fabric may be used in a continuous machine for making artificial board.

Numerical 20 indicates a Fourdrinier or forming wire or screen on which the wet fiber mat 21 is formed and on which it is yet quite plastic through the retention of water. This screen runs along over supporting rolls 22, then through a set of heavier press rolls 23 and 24, lighter press rolls 26 and 27, heavy squeeze rolls 28 and 29, and a second set of squeeze rolls 30 and 31. The wire returns over the lower roll 30, and the moist or damp fiber layer 32 is quite self-supporting, and ready to be dried. As the plastic mat 21 enters these rolls it receives on its top a stretch of an endless impression carrier 33 according to this invention, and an endless thick felt 34 which takes up water squeezed out. Rolls 31, 35 and 36 carry the felt 34. Rolls 31, 35, 37, 38, 39, 40 and 41 carry the impression blanket. Roll 39 depresses the blanket into washing tank 42, so that it may be cleaned of adherent fiber to assure clean impressions. A press roll 43 over roll 38 squeezes excess water out before the blanket is used again. At the roll 31 the loose impression material is removed from the permanent

impressions now set in the mat. Then the board goes to drier 44.

In the manufacture of board as described in the machine of Fig. 4, it is obvious that the felt 34 may itself provide the carrier generally described without departing from the invention. A separate carrier is preferred for many reasons. It is also to be understood that in many board-making machines there is used a top-wire as well as the lower forming-wire. The top-wire also may be used as the carrier for the present invention.

It is further to be understood that I have described the invention in terms of "carrier" and "loose elements" in order to explain clearly the different and specific functions. But it is to be understood that the elements and functions may be merged without departing from the spirit and scope of the invention. For example, referring to Fig. 2, I have described a taut set of strands 10, and a loose set of strands 17. Both sets may be identical strands. One or more strands may belong to set 10 at one part of the structure to function as a carrier, and belong to set 17 at another part of the structure to function as a mobile element. It is therefore to be understood that the invention in its broadest aspect provides a marking structure which as a whole is capable of being pulled in a taut relation to fix the position of the fixations of the mobile elements, so as to present mobile elements for self-positioning. The pattern designed, and the questions of construction with ease and economy determine the exact construction of the device.

It is of course to be understood that a single length (not an endless belt) of impression blanket, may be used where a non-continuous process is used. For example, it may be used in the press shown in U. S. Ziska Patent No. 1,690,152, which is used in an intermittent operation in making artificial board, serving at the same place as the press rolls above described.

In the preferred operation of the process, the wet board marked as above described, is dried by the use of a drier which has hot flattening or pressing means. These operate to reduce the higher spots to the same level, giving a uniform caliper to the board. The depth of the depressions in the surface from the caliper surface has a great effect upon the appearance of the board for ornamental effect. When the depressions are of depth of about 0.02 inch, the depression becomes capable of indicating high lights and shadows on proper lighting, such as any wall is normally subjected to. This is practically the minimum depth, but of course, the high lights and shadows depend upon a rather abrupt drop in the surface from the caliper level or any lower general level, adjacent the depression. It is the form of the depression and the size and depth as well, which are factors to give this effect.

For a board involving the present invention the depth of the depressions may vary from .005 to .04, with a predominant number of them from .02 to .04 inch deep to give high lights. The width of the depressions may vary up to twice the depth to give the high lights and shadows, and preferably the width is not greater than the depth.

The board with the design illustrated is particularly useful for wainscot, with the lines of the pattern running vertically. In such use it is subjected to considerable scuffing. Therefore, it is desirable to increase its utility by

hardening the surface. This may be done by a coat of paint, varnish or other substance applied to the dry board. It may also be done by applications of suitable coating to the wet impressed mat before drying. Such coatings may contain pigments to cover the fibers, as described in the copending applications which may later be referred to. These include aqueous base coats of pigments and binder, which binder may be protein, resinous, starch, or other suitable substance. However, the board may be coated with a non-pigment material effective to harden the surface of the board.

For example, a drying oil may be applied in the form of an oil emulsion, under conditions to induce drying or hardening of the surface while the processing of the board is being completed. By incorporating a drying oil and a drier in an aqueous emulsion, the emulsion may be spread onto a wet mat which ultimately provides the board with the oil limited to and concentrated in the surface layer of the board. Thus, the wet mat before or after the making of design impressions, is treated with such an emulsion, so that in hot pressing the board the oil is hardened while the fibers are still wet in the core of the board, thus concentrating the oil at the surface as a hard surface layer of dried oil embodying the surface fibers. Such a surface is resistant to scuff, marring, spotting with water, and washing with soap and water. It has essentially the surface properties of a paint film, but the surface appearance of a fibrous wallboard. These characteristics depend upon the distribution of the oil in the fibers. By applying oil emulsions to wet fiber mats, the desired oil-type surface, as distinguished from fiber surface begins at about 7 pounds of oil to 1000 sq. ft. of board at 16 pound density per cu. ft. It may be applied up to 30 pounds per 1000 sq. ft. and in practice from 11 to 22 pounds of China-wood oil is used for such wood fiber boards.

A suitable emulsion is as follows:

|                       | Per cent<br>by weight |
|-----------------------|-----------------------|
| Water                 | 69.4                  |
| China-wood oil        | 27.8                  |
| Japan drier           | 2                     |
| Sodium carbonate      | .4                    |
| Dyestuffs (for color) | .4                    |

The sodium carbonate and water at 90° to 110° F. are used as a liquid vehicle to which the mixed and oil are added with emulsifying agitation. Not only the vegetable drying oils such as China-wood oil, soya bean oil, linseed oil, perilla oil, oiticica oil and others may be used, but also the synthetic drying oils produced from non-drying vegetable oils and from petroleum and other hydrocarbon bases. By the term drying oil as used herein is meant any oil not miscible with water which by oxidation, with or without a drier, will form a solid substance, as in paint.

The oil emulsion may be used before or after the impressing of a design into the board, so long as it is applied while the board is wet. The oil particles of the emulsion are thus filtered out by the fiber at or near the surface. In drying the board by heat, the surface is dried before the interior, and the oil is quickly set at the surface. The quick action on the oil before drying the board on the interior limits penetration of oil, making a small amount very ef-

fective to harden the surface for a depth sufficient to give a case-hardened effect.

The oiled surface design face is an excellent base for applying paints, varnishes, lacquers and other finishing compositions. The oil serves to prevent penetration of such materials.

Where design impressions are made in the wet mat, the surface of the board is a continuous felt, to be distinguished in appearance and utility from a finished board of which the natural surface felt is cut to make a design.

The present application is a continuation in part of my application, Serial No. 220,355, filed July 20, 1938. The subject matter relating to the use of drying oil is described and claimed in my application Serial No. 317,105, filed February 3, 1940.

It is of course to be understood that the same method and impression material may be used in cement, plasterboard, gypsum board, and other temporarily plastic body-materials having a decorative surface. These are impressed while plastic, partially set to hold the impressions, and then completely set after removal of the impression-making means.

The invention obviously is not limited to surfacing fiber boards, but may be used on any plastic material. Therefore the invention is broadly defined in the appended claims.

I claim:

1. An artificial decorative board for use on walls and the like in position subject to marring or scuffing having a surface of felted fibers with intaglio markings therein, the felted connection of the fibers of said surface being unbroken by the depressions of the markings, said continuous felt of surface fibers embodying a dried oil, the main body of the board beneath said surface being softer and being free from dried oil, the depressions being in the nature of grooves from .005 to .04 inch deep, the width of a groove being not more than twice the depth, the major portion of the high spots between the said grooves being substantially in the same plane, whereby a flat surface is provided with decorative high lights and shadows upon illumination.

2. An artificial decorative board for use on walls and the like in position subject to marring or scuffing having a surface of felted fibers with intaglio markings therein, the felted connection of the fibers of said surface being unbroken by the depressions of the markings, the depressions extending in the same general direction, said continuous felt surface fibers embodying a hardening agent, the main body of the board beneath said surface being softer than said surface layer and being free from said hardening agent, the depressions being in the nature of grooves from .005 to .04 inch deep, the width of a groove being not more than twice the depth, the major portion of the high spots between the said grooves being substantially in the same plane, whereby a flat surface is provided with decorative high lights and shadows upon illumination.

3. An artificial decorative board for use on walls and the like in position subject to marring or scuffing having a surface of felted fibers with intaglio markings therein, the felted connection of the fibers of said surface being unbroken by the depressions of the markings, the depressions extending in the same general direction, said continuous felt of surface fibers embodying a dried oil, the main body of the board beneath said surface being softer and being free from dried oil, the depressions being in the nature of

grooves from .005 to .04 inch deep, the width of a groove being not more than twice the depth, the major portion of the high spots between the said grooves being substantially in the same plane, whereby a flat surface is provided with decorative high lights and shadows upon illumination.

4. An artificial decorative board for use on walls and the like in position subject to marring and scuffing comprising a body of felted fibers having a surface with intaglio markings therein, the felted connection of the fibers of said surface being unbroken by the depressions of the markings, and dried oil in the surface layer as a hardening agent, the main body of the board beneath said surface being softer than said surface layer and being free from said dried oil.

5. An artificial decorative board for use on walls and the like in position subject to marring or scuffing comprising a body of felted fibers having a surface with intaglio markings therein, the felted connection of the fibers of said surface being unbroken by the depressions of the markings, and dried oil in the surface layer as a hardening agent, the main body of the board beneath said surface being softer than said surface layer and being free from said dried oil, the high spots of the markings being flat and lying in substantially the same plane.

HENRY E. WALTER.

CERTIFICATE OF CORRECTION.

Patent No. 2,317,504.

April 27, 1943.

HENRY E. WALTER.

It is hereby certified that error appears in the printed specification of the above numbered patent requiring correction as follows: Page 3, first column, line 31, for "wshing" read --washing--; line 54, after "mixed" insert --drier--; and second column, line 70, claim 3, for "degressions" read --depressions--; and that the said Letters Patent should be read with this correction therein that the same may conform to the record of the case in the Patent Office.

Signed and sealed this 8th day of June, A. D. 1943.

(Seal)

Henry Van Arsdale,  
Acting Commissioner of Patents.